

# United States Patent Office

3,211,618

Patented Oct. 12, 1965

1

3,211,618

## BASE FOR COSMETICS

Helene Kambersky, Hegelgasse 6, Vienna, Austria  
No Drawing. Filed June 26, 1961, Ser. No. 119,270  
Claims priority, application Austria, July 8, 1960,

A 5,282/60

10 Claims. (Cl. 167—85)

This invention relates to a base for a cosmetic, particularly a cosmetic for eyelashes and eyebrows.

It is known from Austrian patent specification No. 142,033 to use aqueous wax emulsions containing a volatile oil, such as turpentine, for such cosmetics. In Austrian Patent No. 159,218 it is proposed to add a volatile constituent consisting of an ester of a volatile acid, e.g., formic acid ester.

Whereas these cosmetics have good adherence because the volatile substances evaporate soon after application to leave a fine water-insoluble film, the turpentine content of about 50%, which was required, involved the disadvantage that the turpentine in such high concentration had a strong odor and was not tolerable by sensitive persons owing to its known irritating effect on the skin. In Austrian patent specification No. 188,854 it was proposed to add a drying oil, such as linseed oil, and a fatty oil, such as castor oil, to an aqueous emulsion of wax and turpentine. This enables a reduction of the content of turpentine to less than one half of the amount previously required without reducing the suppleness and adherence of the cosmetic. Nevertheless, the odor and sometimes also the irritating effect of turpentine was still a disadvantage when the same was used even in smaller amounts.

It has now been found that an excellent base for cosmetics, particularly for mascara and eyebrow paint, can be obtained on the basis of aqueous wax emulsions if the previously used turpentine is replaced by a mixture of linear paraffins of highest purity and free of aromatics, particularly of isoparaffins having a boiling range between about 160° C. and about 200° C. A mixture which has proved particularly suitable comprises isoparaffins of highest purity, having a boiling range of about 180° C. and about 190° C., which can be obtained by catalytic processes from cracked gases and other low-boiling petroleum hydrocarbons and is available, e.g., under the trade name "Shellsol-T."

These products consist of a colorless, highly fluid, oily liquid which is odorless and chemically inert. They are distinguished from turpentine by having a beneficial effect on the skin. There is no irritation experienced whatever. When a cosmetic prepared with these products has been applied, e.g., to the eyelashes, moreover the cosmetics will dry within a few minutes to form a non-smearing, firmly adhering, moisture-resisting film.

It has been found that when the components of the cosmetic are emulsified in the usual manner, the paraffins provided according to the invention together with an emulsifier, the desired pigments and perfumes and, if desired, a substance acting as an odor carrier, such as terpineol, give a homogeneous emulsion of excellent quality. Suitable emulsifiers include, above all, mixtures of higher fatty alcohols and/or fatty alcohol sulfonates, such as the products known under the trade name "Lanette Wax."

The base for cosmetics according to the invention contains preferably about 10–60% paraffins, depending on the desired consistency of the cosmetic. Owing to the ease with which these paraffins can be emulsified, and because of their odorlessness and harmlessness, the paraffins may be used in such large quantities that it is possible, as contrasted with the use of turpentine, to make a cosmetic, e.g., a mascara, in semiliquid form. Such a cos-

2

metic has the advantage that it can be applied easily and in a very thin layer. Besides, it is more economical in consumption than the previous, thicker emulsions, which adhere to the tube walls so that when the contents of the tube are gradually consumed, part of it always remains in the tube without utilization, whereas the more fluid product can easily be squeezed out of the tube and be entirely removed therefrom.

The base for cosmetics according to the invention may desirably contain small additions of a drying oil and/or a fatty oil. The presence of a drying oil, such as linseed oil, promotes a rapid drying of the cosmetic on the surface to which it is applied and prevents a subsequent smearing or sticking together of eyelash hairs. The fatty oil, such as castor oil, improves the suppleness and supplies a nutritive substance to the skin.

The quantitative proportions of the components may lie within the following limits:

|    | Percent by weight                               |
|----|-------------------------------------------------|
| 20 | Wax (beeswax, ceresine or the like) ----- 20–30 |
|    | Paraffin mixture ----- 10–60                    |
|    | Emulsifier (such as Lanetta Wax N) ----- 5–10   |
|    | Water ----- 10–40                               |
| 15 | Drying oil, such as linseed oil ----- 0–5       |
| 25 | Fatty oil, such as castor oil ----- 0–8         |

In the following examples, specific compositions of the base for cosmetics according to the invention are disclosed, whereas the invention is not restricted thereto.

|    | Example 1                                                                                 | Percent by weight |
|----|-------------------------------------------------------------------------------------------|-------------------|
|    | Beeswax ----- 20                                                                          |                   |
| 35 | Shellsol-T (isoparaffin mixture boiling point between 180° C. and about 190° C.) ----- 60 |                   |
|    | Castor oil ----- 2                                                                        |                   |
|    | Lanette Wax ----- 5                                                                       |                   |
|    | Water ----- 13                                                                            |                   |

|    | Example 2              | Percent by weight |
|----|------------------------|-------------------|
|    | Beeswax ----- 30       |                   |
| 40 | Shellsol-T ----- 12    |                   |
|    | Castor oil ----- 8     |                   |
| 45 | Lanette Wax N ----- 10 |                   |
|    | Water ----- 40         |                   |

|    | Example 3              | Percent by weight |
|----|------------------------|-------------------|
| 50 | Beeswax ----- 25       |                   |
|    | Shellsol-T ----- 30    |                   |
|    | Lanette Wax N ----- 10 |                   |
|    | Water ----- 35         |                   |

|    | Example 4              | Percent by weight |
|----|------------------------|-------------------|
| 55 | Beeswax ----- 26       |                   |
|    | Shellsol-T ----- 30    |                   |
|    | Castor oil ----- 5     |                   |
|    | Linseed oil ----- 4    |                   |
| 60 | Lanette Wax N ----- 10 |                   |
|    | Water ----- 25         |                   |

I claim:

1. A base for a mascara, comprising an aqueous emulsion containing, by weight, about 20–30% wax, about 10–60% of a mixture of linear paraffins substantially free of aromatics, which mixture has a boiling range between about 160° C. and about 200° C., about 5–10% of an emulsifier selected from the class consisting of higher fatty alcohols, higher fatty alcohol sulfonates and mixtures thereof, and about 10–40% water.

2. A base as claimed in claim 1, which contains up to 5 percent by weight of a drying oil.

3. A base as claimed in claim 1, which contains up to 10 percent by weight of a fatty oil.
4. A base as claimed in claim 1, which contains up to 5 percent by weight of a drying oil and up to 10 percent by weight of a fatty oil.
5. A base as claimed in claim 1, in which said wax comprises beeswax.
6. A base as claimed in claim 1, which contains up to 5 percent by weight of linseed oil.
7. A base as claimed in claim 1, which contains up to 10 percent by weight of castor oil.
8. A base as claimed in claim 1, which contains up to 5 percent by weight linseed oil and up to 10 percent by weight castor oil.
9. A base as claimed in claim 1, which said mixture consists of isoparaffins.
10. A base as claimed in claim 9, in which said mixture has a boiling range between about 180° C. and about 190° C.

## References Cited by the Examiner

## UNITED STATES PATENTS

2,566,716 9/51 Boe ----- 260—17

5

## FOREIGN PATENTS

208,806 6/57 Australia.

## OTHER REFERENCES

Bennett, Commercial Waxes, Chem. Pub. Co., New York, 1956, pp. 509, 537, 604, 611.

Shellsol T, Shell Oil Co., New York, booklet pp. 1-3, February 1961.

Zimmerman et al., Handbook of Material Trade Names Industrial Research Service, Dover, N.H., Supp. 1 to 1950 Ed. (1956), pp. 213-214.

JULIAN S. LEVITT, Primary Examiner.

MORRIS O. WOLK, LEWIS GOTTS, Examiners.